

## UNITED STATES PATENT OFFICE

2,375,446

## RESISTANCE OR FUSE WIRE

Cecil Spencer Sivil, Roselle, N. J., assignor to  
 Baker & Company, Inc., Newark, N. J., a corporation of New Jersey

No Drawing. Application July 8, 1943,  
 Serial No. 493,946

3 Claims. (Cl. 201—76)

This invention deals with electrical resistance wires and is concerned in particular with electrical resistances suitable for instance in the ignition of explosives such as fuse or bridge wires in blasting caps, detonators, or the like.

Heretofore such resistance wires for igniting or setting off explosives usually consisted of an alloy of platinum-iridium containing from 10% to 20% iridium, the alloy of 80% platinum and 20% iridium generally being preferred. Because of the high cost of such alloys attempts have been made to cheapen the cost of such wire by substituting part or all of the precious metal with base metals, resulting however in the production of wires which tended to corrode under the influence of the atmosphere or the match compounds in which they were embedded, which made such wires unfit for use unless used reasonably soon after production of the wire or insertion in the fuse. Other attempts to replace all or part of the expensive iridium in such platinum-iridium alloys have been made, but such attempts were limited to the incorporation or substitution of other high priced precious metals and thus did not afford satisfactory relief from the high cost of the platinum-iridium alloy resistance wires for fuses.

It is one object of my invention to produce a resistance wire for use in igniting explosives, as in blasting caps, detonators or the like, which shall consist substantially of precious metals only and shall have low specific gravity, high electrical resistance and satisfactory breaking loads or tensile strength to take the place of fuse wire of platinum-iridium alloys heretofore in general use in setting off explosives, and which while having characteristics similar to those of such platinum-iridium wires shall be of considerably lower cost. It is another object of this invention to provide a platinum metal electrical resistance wire for other uses requiring electrical resistance and corrosion resistance. Other objects of the invention will appear from the description thereof herein-after following.

This application is a continuation in part of my earlier application Serial No. 288,572 filed August 5, 1939.

I have discovered that electrical resistance wires such as fuse wires achieve the hereinbefore stated objects when constructed of alloys of platinum

5 palladium and at least one metal of the group ruthenium and rhodium, in particular ruthenium. The alloys utilized and found suitable for the purpose contain from 10% to 80% platinum, from 12% to 89% palladium, and from 1% to 15% of at least one metal of the group consisting of ruthenium and rhodium. The electrical resistance wires of the invention can be divided into two groups. One group has a relatively high platinum content and correspondingly low palladium content, such as alloys containing from 60% to 80% platinum, from 12% to 30% palladium, and from 1% to 15% ruthenium, such for instance as alloys of 65% platinum 25% palladium 10% ruthenium, or of 70% platinum 24% palladium 6% ruthenium, or of 74% platinum 20% palladium 6% ruthenium, or of 80% platinum 14% palladium 6% ruthenium. The other group has a relatively low platinum content and correspondingly high palladium content such as alloys containing from 10% to less than 60% platinum, preferably not more than about 55% platinum, from more than 25% palladium to 89% palladium and from 1% to 15% ruthenium or rhodium, such for instance as alloys of 55% platinum 30% palladium 15% ruthenium, or of 55% platinum 35% palladium 10% ruthenium, or of 50% platinum 47% palladium 3% ruthenium, or of 40% platinum 57% palladium 3% ruthenium, or of 30% platinum 67% palladium 3% ruthenium, or of 20% platinum 77% palladium 3% ruthenium, or of 10% platinum 87% palladium 3% ruthenium.

20 In all cases the platinum content must not fall 35 below 10% and should not exceed 80%, and while the palladium content should not fall below 12% and must not exceed 89% it should preferably exceed 25% and comprise in particular at least 30%. The ruthenium content, like the rhodium content, must not fall below 1% nor exceed 15% and preferably runs from 3% to 10%. The most suitable and advantageous fuse wire is constructed of alloys of 25% to 55% platinum, 30% to 74% palladium, and 1% to 10% ruthenium, and shall 40 be of alloys of 40% to 55% platinum 45% to 59% palladium and 3% to 10% ruthenium. In particular I recommend an electrical resistance wire of about 47% platinum about 57% palladium about 3% ruthenium.

45 The following table will illustrate some of the

properties of the electrical resistance wires of the invention, the table showing comparative data for electrical resistance wires of 80% platinum-20% iridium alloy and certain electrical resistance wires of the invention with high platinum and low palladium content on the one hand and low platinum and high palladium content on the other hand.

| Composition, per cent |    |    | Breaking load, grams at 300 ohms/yd. | Resistivity ohms/mil. ft. | Density gr./cc. | Melting point, °C. |
|-----------------------|----|----|--------------------------------------|---------------------------|-----------------|--------------------|
| Pt                    | Ir |    |                                      |                           |                 |                    |
| 80                    | 20 |    | 110-120                              | 200                       | 21.6            | 1,950              |
| Pt                    | Pd | Ru |                                      |                           |                 |                    |
| 10                    | 87 | 3  | 70                                   | 153                       | 12.6            | 1,575              |
| 20                    | 77 | 3  | 74                                   | 169                       | 13.2            | 1,595              |
| 30                    | 67 | 3  | 76                                   | 190                       | 13.9            | 1,620              |
| 40                    | 57 | 3  | 77                                   | 200                       | 14.5            | 1,640              |
| 50                    | 47 | 3  | 83                                   | 212                       | 15.4            | 1,660              |
| 60                    | 37 | 3  | 90                                   | 220                       | 16.4            | 1,680              |
| 70                    | 24 | 6  | 140                                  | 250                       | 17.3            | 1,700              |
| 74                    | 20 | 6  | 128                                  | 243                       | 17.8            | 1,710              |
| 80                    | 14 | 6  | 70                                   | 235                       | 18.5            | 1,730              |

Platinum palladium ruthenium and rhodium are, like iridium, members of the platinum group and possess considerable corrosion resistance. Palladium as well as ruthenium and rhodium has a specific gravity considerably lower than that of either platinum or iridium and the electrical resistance wires of the invention possess, therefore, a lower density than the electrical resistance wire of platinum iridium alloy. In the high platinum content alloy wires of the invention the tensile strength and electrical resistance are higher than in the low platinum content alloy wires of the invention. All resistance wires possess high corrosion resistance as required in the case of fuse wires.

The electrical resistance wires of relatively low platinum and high palladium content represent particularly desirable electrical resistance wires in that they have an especially low specific gravity. They contain considerably less platinum than the platinum iridium wires of the prior art and while they possess less tensile strength and lower electrical resistance than either the platinum iridium wires of the prior art or the wires of the invention having a high platinum content they will have sufficient tensile strength for the purpose and the particular electrical resistance of the individual wires can be controlled by varying the diameter of the wire. Fuse or bridge wires for blasting caps for instance usually have an electrical resistance of 300 ohms per yard. A fuse wire of 80% platinum-20% iridium alloy possessing such resist-

ance has a diameter of 0.0015". A fuse wire of 40% platinum 57% palladium and 3% ruthenium, representing the best embodiment of electrical resistance wires of platinum palladium ruthenium alloy having a low platinum content, has such resistance of 300 ohms/yd. when the wire is given a diameter of 0.0014". Whenever, therefore, the electrical resistivity in terms of ohms/mil. ft. is lower for any alloy within the scope of the invention than for 80% platinum-20% iridium the same ohms/yd. resistance can be obtained by decreasing the diameter of the wire, and vice versa, so that in actual practice electrical resistance wires can be produced from the range of alloys stated identical with that of a fuse wire of 80% platinum-20% iridium alloy now in use. The breaking load of the individual wires, while lower than that of the prior art wire of 80% platinum-20% iridium alloy, is, nevertheless, sufficient for the purposes contemplated, particularly where the platinum content does not fall below about 25%. While one ounce of 80% platinum-20% iridium alloy will furnish only 4520 ft. at 300 ohms/yd., one ounce of 87% palladium-10% platinum-3% ruthenium alloy will furnish 10,500 ft. at 300 ohms/yd., and one ounce of 57% palladium-40% platinum-3% ruthenium will furnish 7300 ft. at 300 ohms/yd. On the other hand, for instance, a wire of 70% platinum 24% palladium and 6% ruthenium will have an electrical resistance of 300 ohms/yd. when it is given a diameter of 0.0016", in which case 1 ounce of alloy will furnish 4535 ft. of wire.

The electrical resistance wire may be used wherever a corrosion resistant wire is desired for the purpose of resisting the passage of an electrical current or producing a potential drop of some desired amount. Although it is specifically designed for use as a fuse or bridge wire for the setting off of explosives, it may also be used for instance as resistance wire in the Wheatstone bridge, as in gas analyzers or the like.

What I claim is:

1. Electrical resistance wire of an alloy of platinum palladium and ruthenium comprising from 25% to 55% platinum, 30% to 74% palladium, and 1% to 10% ruthenium.

2. Electrical resistance wire of an alloy of platinum palladium and ruthenium comprising from 40% to 55% platinum, 45% to 59% palladium, and 3% to 10% ruthenium.

3. Electrical resistance wire of an alloy of platinum palladium and ruthenium comprising about 40% platinum, about 57% palladium, and about 3% ruthenium.

CECIL SPENCER SIVIL.